

## UNITED STATES PATENT OFFICE

JOHN C. WATSON, OF ATTLEBORO, MASSACHUSETTS, ASSIGNOR, BY DIRECT AND MESNE ASSIGNMENTS, TO B. B. & R. KNIGHT CORPORATION, OF PROVIDENCE, RHODE ISLAND, A CORPORATION OF RHODE ISLAND

## CROSS-DYEING CELLULOSE FABRICS

No Drawing.

Application filed July 20, 1926. Serial No. 123,801.

My invention relates to an improved process of manufacturing an all cellulose textile fabric in contrasting colors. I employ the words "cellulose textile fabric" to include an 5 all cotton fabric, or a fabric made from the type of rayons which contain substantially the same percentage of cellulose as cotton or a greater percentage of cellulose and which have substantially the same affinity for the 10 same types of dyestuffs as cotton namely, viscose rayon, cupraammonium rayon and chardonet rayon, etc., entirely or mixed with cotton. This application is a continuation in part of application #73,471, filed Dec. 5, 15 1925, which discloses broadly the same invention as this application. There is filed of even date herewith a second application Serial No. 123,802; a continuation of application #94,089, filed Mar. 11, 1926 covering 20 specifically a second species of the broad invention disclosed in this application and another application covering a third species of the invention, Serial #123,803, filed of even date herewith, July 20, 1926.

25 Hitherto where it has been desired to produce a fabric having a two color effect, either the warp or the filling have been woven of two different materials such as cotton and silk, which will take the dye in different shades or 30 amounts, or the warp or filling yarns have had to be separately dyed with two different colored dyes prior to weaving.

The main feature of my process is to treat 35 the warp during the slashing process with the first step of a two step dyeing process, the nature of the ingredient thereof added to the size being such that it will have no appreciable effect upon the functioning of the size, nor will the size have any appreciable effect 40 upon its functioning, weaving the cloth in the usual manner with a filling and later treating the fabric with the second step of a two step dyeing process, which acts upon the prepared warp to form the dye thereon. I am aware that hitherto it has been suggested to 45 add a direct or substantive dye to the size to simultaneously size and dye the fabric with a one step dyeing process. As the actual water soluble dye has to be inserted with the 50 size it is obvious that in a short space of time,

the size bath will become messy and the dyeing irregular and in addition a fast color is not produced. Various types of two step dyeing processes are known and it is immaterial for the purposes of my invention what 55 type of a two step dyeing process be employed so long as one is chosen wherein the first step has no appreciable effect upon the functioning of the size, nor the size on its functioning. The types of two step dyeing 60 processes however, may be generally classed as three, namely (A) where the first step thereof consists of treating the warp with a water soluble chemical having non-dyeing 65 properties such as an organic or inorganic mordant or a soluble mineral salt and the second step treating it with a dye. (B) where the first step consists of treating it with a dye or a dye component and the second step consists of treating it with an additional 70 dye component and (C) where the first step consists of treating the warp with a dye-stuff in a true or modified form and the second step consists of treating it with a chemical having an oxidizing or a reducing action. 75 The subject matter of species A is specifically claimed in this application, namely, where a chemical is inserted with the size and the dye ingredient applied to the entire fabric to combine only with the treated warp. 80

I am aware that cotton goods of contrasting colors have been made by treating the warp or the filling threads entirely independently of the slashing process with a tannin mordant before weaving the cloth in the usual manner with an unprepared filling and then dyeing the fabric with a basic color which acts upon the mordanted warp alone and later dyeing the fabric with a direct color which acts on the unmordanted filling. This process is impractical and expensive for two reasons: it requires the extra cost of an entirely distinct and separate step such as mordanting independently of any sizing and prior to weaving of suitably treating the proper threads with the first step of a two step dyeing process. Thus the added cost of this added step makes this method of dyeing impractical. The warp is first beamed in a suitable fashion for use in a loom and then passed 100

through a slasher box to cover it with a size so that the individual warp threads will stand up during the friction and wear they receive in the weaving process, the fabric is, then woven in the usual manner. Thus in the usual gray cloth manufacturing plants at present there is no suitable dyeing or mordanting apparatus for performing this separate step. Employing my process however, which merely consists in putting a small amount of the ingredient of the first step of a two step dyeing process right into the slasher, a piece of standard equipment in every cotton mill, it is obvious that my process can be employed without the necessity of purchasing extra dyeing or mordanting equipment or without turning the cotton mill into a dye house. After weaving the fabric in the gray form it may then be sent to the dye house where the rest of my process may be completed to dye the fabric in contrasting colors with the usual dyeing equipment by any of the well-known processes.

These and such other objects of my invention as may hereinafter appear will be best understood from a description of various embodiments of my process.

My invention includes simultaneously treating the warp threads in the slashing process with a suitable size for weaving and with a first ingredient of a two step dyeing process, each of which has no appreciable effect on the functioning of the other, weaving the cloth in the usual manner with a filling and then treating the entire fabric with the second step of a two step dyeing process which acts upon the prepared warp to form the dye thereon. If desired the filling may be left white or it may also be dyed by again dyeing the fabric with a dye of a different nature and color, which acts on the filling to dye it a contrasting color to the warp. Whether the filling be left white or dyed it is obvious that it will always be of a contrasting color to the dyed warp.

As stated it is immaterial what type of a two step dyeing process be employed and a two step dyeing process may be selected wherein the first step thereof comprises treating the warp with an ingredient which is neither a dye nor a dye component, but merely a certain type of water soluble chemical having nondyeing properties, weaving the cloth with a filling and then treating the entire fabric with the second step of a two step dyeing process which in the generic sense of my broad invention, may comprise a dye or a dye component. It is obvious that various types of well-known two step dyeing processes may be included in this class, as where the first step comprises applying a mordant to the warp and the second step comprises applying a dye to the fabric. A species of this class which is the species specifically claimed in this application comprises adding an or-

ganic mordant to the warp with the size and a basic color to the fabric after weaving. Also there may be included in this class the precipitation of mineral pigments in the cloth as is usual in khaki dyeing, namely, applying a soluble mineral salt with the size to the warp and forming the color by later precipitating the pigment by treating with an hydroxide.

I will now describe the embodiment of my invention specifically claimed in this application, which consists in dyeing the warp with a basic color. The slashing or size tank is filled up to the usual working level with the following material in approximately the following proportions,—

25 pounds sago flour or any other suitable starch or sizing material dissolved in 50 gallons of water by boiling it twenty minutes; then if desired 2 gallons alizarine oil may be added, then a solution of 20 pounds of tannic acid and 10 gallons of hot water may be added to the size solution. It is understood that in place of sago flour, any suitable starch or sizing material in proportions depending on the result desired may be employed and that in place of tannin, any other mordant, if a basic dye is to be employed an organic mordant, which has no appreciable effect on the size, and the size on it, may be employed. After the size and mordant have been mixed thoroughly and run into the slasher box, the warp is threaded through the mixer in the slasher box in the usual fashion, then through the usual squeeze rolls, around the usual drying cans and on to the usual beam where it is conveniently beamed and then put aside for use in the loom.

The cloth is then woven with the mordanted and sized warp and preferably an unprepared filling. If desired, however, the filling may be dyed or otherwise prepared. The now complete gray cloth is then shipped to the dye house.

After arrival at the dye house the fabric is then treated in any of the usual manners, preferably for one-half an hour in the jig with a solution of an antimony salt which may consist of  $\frac{1}{2}$  ounce per gallon to fix the tannic acid or other mordant on to the warp threads, the time and nature of the treatment depending on the effect to be produced. The fabric is then preferably well washed, preferably given two runs through a warm solution of alum, about two ounces to the gallon, then again washed. After this later washing, the fabric is dyed in the usual manner with a basic dye, preferably with a 3 to 4 percent solution thereof, which basic dye as is well-known acts upon the mordanted warp alone and has no appreciable effect upon the filling. Thus if it is desired to dye the warp a blue, it may be dyed in a bath containing a 4% solution of methylene blue, or a pink, a 4% solution of rhodamine pink, the strength of the solution depending upon

the color desired. Then, if it is desired to mercerize the goods, they may be dried, singed, mercerized in the usual fashion, scoured and washed. If it is not desired to 5 mercerize the goods, and if mercerized after the last wash, the second color is merely put on the filling by dyeing the entire fabric preferably with a direct or substantive dye of a contrasting color or shade in any of the 10 usual manners, preferably with a 3 or 4% solution thereof, the strength, however, depending upon the shade desired. The direct color may be put upon the filling in any one of the well known processes, preferably in 15 a jig. If no mercerizing is done, the goods already being in the jig, it is merely necessary to draw off the basic dye bath, wash the goods, give them a light soaping and put in the direct dye to form a new bath in the 20 same jig. The goods may then be washed, dried, and finished in the usual manner. If it is desired to have the filling threads undyed, or left white a contrasting color to the dyed warp, the last step of dyeing the 25 fabric with a direct color may be dispensed with. In place of an organic mordant, it is obvious that an inorganic mordant may be inserted in the size and the goods dyed later with other types of suitable dyes besides basic 30 dyes. Thus, if desired, the acetates or hydroxides of aluminum, iron or chromium may be inserted with the size and after weaving the goods, they may be treated with a suitable fixing agent and then dyed with a 35 suitable dye such as alizarine to dye the warp. It is obvious that in place of a mordant any type of a dye preparatory chemical may be employed. Where it is desired to impregnate a pigment on the fabric as is done in khaki 40 dyeing a soluble mineral salt, as ferric chloride, acetate of iron, or acetate of chromium may be the ingredient of the first step and after weaving the goods, they may be after-treated in a caustic soda or other hydroxide 45 solution to impregnate the fabric with a basic hydroxide of iron, chromium etc., the actual pigment or dyestuff of dyes of this description, as is well known, the basic hydroxide of chromium giving a green and the basic 50 hydroxide of iron giving a yellow. As stated hitherto, although my process is claimed generically in this application the type of two step dyeing process specifically claimed herein only includes those wherein the first 55 step of the process comprises inserting with the size a water soluble chemical or other ingredient having nondyeing properties, which may not strictly speaking, be termed a dye or a dye component.

60 It is obvious however that a two step dyeing process may be selected wherein the first step thereof normally comprises treating the warp not with a water soluble chemical having nondyeing properties, but with a real dye 65 ingredient or a dyestuff in a true or modified

form or an intermediate dye component, which would have no appreciable effect on the size, nor the size on its functioning. So far as I am aware no one has hitherto conceived of manufacturing an all cellulose 70 textile fabric having component sets of warp and filling threads of contrasting colors by treating before weaving one of said component sets of threads with a dye ingredient of a two step dyeing process at any stage in 75 the preparation of said set, then weaving said component set with the other component set to form the cloth and then impregnating the dyestuff on the prepared component set by treating the fabric with the second step of the 80 two step dyeing process, which acts upon the prepared component set to impregnate the dye thereon. The other component set may be either left white in a contrasting color to the dyed component set or dyed in a contrasting color by again separately dyeing the 85 fabric with a dye of a different nature and color which acts on the unprepared set to dye it a contrasting color to the prepared component set. If desired each component 90 set may be treated with a different dye ingredient of a two step dyeing process and the entire fabric subjected to a second common step of the two step dyeing process, which 95 will simultaneously impregnate each component set with a different dyestuff. It is thus obvious that the other component set, normally the one not sized, may be either first dyed or prepared for simultaneously 100 impregnating the dyestuff thereon with the other component set after weaving or left unprepared. My invention is peculiarly adapted to dye the warp threads with a relatively fast color and specifically includes simultaneously treating the warp threads 105 with a size in the slashing process and simultaneously treating them with a dye ingredient of a two step dyeing process in the same solution. This eliminates the extra cost of an entirely distinct and separate step such as treating with a naphthol, namely independently of any sizing and prior to weaving of suitably treating the proper threads with its added cost. At present in the composite 110 process five steps are necessary.

(1) To size the warp.  
 (2) To treat the warp threads with a dye ingredient of a two step dyeing process.  
 (3) To treat the warp threads with the second step of a two step dyeing process.  
 (4) To treat the filling threads with a dye ingredient of a two step dyeing process.  
 (5) To treat the filling threads with the second step of a two step dyeing process.

Employing my invention however, especially where types of napthols, or indigosols later to be described are employed it is obvious that these five steps may be cut down to three, namely, step one of sizing the warp threads, and step two of treating the warp 125

threads with a dye ingredient of a two step dyeing process may be done simultaneously. Step four of treating the filling threads with a dye ingredient of a two step dyeing process will have to be done separately as usual. The sized and prepared warp threads and the prepared filling threads may be then woven and step three namely, treating the warp threads with the second step of their respective two step dyeing process and in addition step five of treating the filling threads with their separate step of their respective two step dyeing process may be done simultaneously by treating the warp and the filling threads in the fabric with the same step.

This class of a two step dyeing process, namely where the first step in the two step dyeing process comprises treating the material to be dyed with a dye or dye ingredient divides itself into two general classes namely

- (a) Where the second step comprises treating the fabric with an additional dye or a dye component and,
- (b) Where the second step in the dyeing comprises treating the material desired to be dyed with a chemical to impregnate the dyestuff on the fabric.

I will now describe in detail various embodiments of these different classes, this entire generic class being claimed in application Serial #123,802 filing date July 20, 1926, signed of even date herewith, a continuation in part of application #94,089, filed March 11, 1926, which specifically claims dyestuffs of the generic sub-class B heretofore referred to. Dyeing with a type of dyestuff hereinafter referred to in sub-class C is specifically claimed in application Serial #123,803 filing date July 20, 1926, signed of even date herewith.

Although as stated, the preparation of either or both of these sets of component threads by treating them with a dye ingredient of a two step dyeing process may be done at any point in the preparation prior to weaving, I preferably so treat the warp threads while slashing and I will specifically describe this treatment in this description of the application of the following dyes. As stated however, it is immaterial whether the filling be first dyed, separately prepared by treating it with a dye ingredient of a two step dyeing process or left unprepared. I will now describe specifically the application of the dyeing process of the type of dyestuffs normally included in classes B and C namely, where the warp is simultaneously slashed and treated with a dye ingredient of a two step dyeing process where that dye ingredient comprises a dyestuff or an intermediate dye component, whether after weaving the entire fabric is after treated with a dye or with an intermediate dye component which couples with said first dye or intermediate dye com-

ponent to form a dyestuff on the prepared warp as in class B or whether the dyestuff be formed on the warp by treating the fabric with a chemical as in class C. Perhaps the most important class of dyestuffs in this general class B are the developed colors. Applying my process to developed colors I simultaneously treat the warp in the slashing process with a size and with an intermediate dye component such as naphthol, each of which has no appreciable effect on the functioning of the other, weave the cloth in the usual manner with a filling and later on after-treating the entire fabric with a second intermediate dye component such as a developed dye base to couple said components to form a dyestuff impregnated on the prepared warp. My invention therefore makes it possible to dye the warp or filling, also if desired in faster shades than hitherto thought possible in cellulose dyeing of this description. The slasher tank solution may be prepared as follows: 25 pounds of sago or other suitable size are added to 50 gallons of water. To this bath is added if desired 2 gallons of alizarine soluble oil. To this bath is also added as an intermediate dye component 6 pounds of naphthol A. S. and 4 pounds of dry caustic soda. These materials may then be boiled together for about twenty minutes in the size tank, after which 5 pounds of sodium thiosulphate crystals are added.

After the contents of the size tank have been mixed well, they are then run into the slasher box and the warp sized as usual. It is thus obvious that the goods may be prepared for dyeing the warp with a developed color merely by adding a small proportion of an intermediate dye component to the sizing mixture. In place of sago, potato, corn or any suitable kind of starch, flour or any suitable sizing material may be employed, and in place of naphthol, caustic soda and sodium thiosulphate, any other suitable dye component with its other necessary ingredients may be employed. The goods are then woven as hitherto explained and are then sent from the weave shop to the dye house.

After weaving, the dye is suitably developed with a diazo base which acts upon the prepared warp. Although this may be done in any suitable manner, it is preferably done in a jig. For this purpose 7 pounds of red base may be dissolved in 8 gallons of boiling water, to which 2 gallons of hydrochloric acid may be added. After standing one-half hour in the mixing tub, a block of ice is inserted therein. After the mixture is cooled to about 40° F. 4½ pounds of sodium nitrite or other suitable chemical is added. After standing one-half hour 4½ pounds of powdered alum are preferably added.

Just prior to use, 7 pounds of powdered chalk are preferably added, when the entire solution may be poured into the jig. The

fabric is then passed through the jig for several minutes, sufficient to thoroughly diazotize and develop the color on the warp. The strength and materials and time of dyeing, of course, depend to some extent upon the shape desired. It is obvious that in place of the red base and other chemicals described, other suitable intermediate dye components or chemicals may be employed depending upon the color or shading desired to be produced. This dye bath is then run off, the goods washed, preferably in the jig, or if desired, dried, singed and mercerized. If not mercerized, after the last wash, the goods may be re-dyed in the same jig preferably with a 3 or 4% solution of a substantive or direct color of a different shade. After this, they may be washed, dried and finished in the usual manner. If it is desired to have the filling threads white in contrast to the dyed warp threads, the last step of dyeing the fabric with a direct color may be dispensed with.

Any suitable type of naphthol may be employed. There have recently come on the market various different types of new naphthols, which are derivatives of naphthol such as the A. S. group, which is probably the best known which are aryl amides of beta-oxy-naphthoic acid. Any of these naphthols may be coupled with a second intermediate dye component to form a dyestuff on the prepared warp. In fact different naphthols of this group may be coupled with the same base or second intermediate dye component to form different colored dyestuffs. Thus, if desired very pretty fast color effects may be produced, such as by treating the warp in the slashing process with a naphthol A. S. S. W. and then treating the filling prior to weaving with a naphthol A. S. G., then weaving the cloth in the usual manner and later after treating the fabric with a fast black L. B. base, a black dye will be developed on the prepared warp and a brownish red dye will be developed on the prepared filling, both dyes of the normal fastness of developed dyes. It is thus obvious that in employing my invention in this manner faster shades may be developed on the filling, than is possible by merely dyeing the filling by after dyeing the entire fabric with a direct or substantive color. It is obvious that in place of naphthol any suitable intermediate dye component may be employed and in place of a red base or a fast black L. B. base any suitable type of a second intermediate dye component may be employed. If desired the stabilized diazo compounds which have recently come upon the market may be employed as the second intermediate dye components which dissolve in water directly to form the coupling solution without the necessity of any other chemicals or treatment. In

place of naphthols or their derivatives any other suitable type of intermediate dye component such as N. W. acid etc. may be employed to be coupled with a diazo component as the second step. If desired an intermediate dye component of the type of primuline may be employed as the first intermediate dye component which when diazotized and treated with a naphthol as a second dye component will develop a fast red color on the treated component set, in a sense a reversal to the method specifically described.

I will now specifically describe the application of class C of the two step dyeing process where the first ingredient of the two step dyeing process comprises treating the fabric with a dyestuff modified or unmodified and the second step thereof comprises after treating the fabric with a chemical having an oxidizing or a reducing action. The most important types of dyestuffs of this class includes vat dyestuffs or their derivatives which as is well-known are among the fastest colors. Any suitable type of vat dyestuffs may be employed. If the vat dyestuff be insoluble it may be adhered to the prepared warp with the size and when the fabric is suitably after-treated after weaving the insoluble vat dyestuff will change into a leuco compound to dye the warp on withdrawal from the bath.

Perhaps the most important class of modified dyes which may be dyed in this manner are the stabilized water soluble derivatives of vat dyestuffs which have recently come on the market. Any suitable type of this general type of dyestuff may be employed. What I preferably employ are the types of dyestuffs described in U. S. Patents Nos. 1,448,251 and 1,575,958 which are the water soluble ester-like derivatives of the leuco compounds of any suitable type of vat dyestuffs whether they be produced from indigo as are the types now being put on the market by Société Durand & Huguenin S. A. or those derived from indanthrenes, which according to an article in "The Journal of Dyers and Colorists" for Feb. 1925 are now being put on the market by the Scottish Dyes Ltd. This class of ester-like derivatives whether they be produced from indigo or from indanthrenes or from any other vat dyestuffs are aftertreated to develop the dyestuff on the fabric by reforming the dye by the action of a suitable oxidizing agent. For the purposes of my invention however, any suitable type of a stabilized water soluble derivative of a vat dyestuff may be employed like the dehydro-indigos as described in German Patents Nos. 217,477—220,173—237, 262—239,814—which are later developed on the fabric by reforming the dye by the action of a suitable reducing agent.

I will specifically describe the application of an indigosol, such as indigosol O. B. for blue sold in America by the General Dye-

stuffs Corporation, specifically applying it to the warp in the slashing process. The slasher tank solution may be prepared as follows: 25 pounds of sago or other suitable size are added to 50 gallons of water. To this bath is added if desired 2 gallons of alizarine soluble oil. To the bath is also added as the dye ingredient of the two step dyeing process 1-3 pounds of indigosol blue O4B the amount depending on the shade desired, preferably previously dissolved in about 3 gallons of water. These materials may then be boiled together for about 20 minutes in the size tank after which an amount of sodium nitrite equal in weight to the indigosol used is added. After the contents have been mixed well they are then run into the slasher box and the warp sized as usual. It is thus obvious that the goods may be prepared for dyeing the warp with a vat color by adding a small proportion of a vat dyestuff, modified, or unmodified to the sizing mixture. In place of sago, potato, corn, or any other suitable starch, flour or any other suitable sizing materials may be employed and in place of indigosol O4B any type of vat dyestuff modified or unmodified preferably a stabilized water soluble ester-like derivative of the leuco compound may be employed. In place of sodium nitrite any suitable oxidizing agent may be employed, or if desired this may be dispensed with. The goods are then woven as hitherto explained and then sent from the weave shop to the dye house.

After weaving, the dyestuff is developed on the warp by suitably forming the dye thereon by any suitable aftertreatment depending on the nature of the vat dyestuff employed. Where an indigosol or any water soluble ester-like derivative of a vat dyestuff has been employed as the first dye ingredient, I preferably reform the dyestuff on the warp by an action of a suitable oxidizing agent. Although this may be done in any suitable manner, it is preferably done by passing the woven fabric through a jig. To reform the dyestuff by oxidation and to free the oxygen from the sodium nitrite preferably added to the first dye ingredient with the size, I preferably fill the jig with a 2° Tw. sulphuric acid, when dyeing with an indigosol or like ester-like derivative the color will immediately be developed on the warp. If other types of vat dyestuffs or their stabilized water soluble derivatives be employed they may be suitably reduced to the desired leuco compound in any well-known manner, after which the dyestuff will be reformed on the fabric by oxidation on exposure to the air. Any suitable type of acid may be employed and any other suitable type of an oxidizing agent other than nitrite of soda may be employed. The goods are then washed, soaked and washed, preferably in a

jig or if desired dried, singed and mercerized. If not mercerized after the last wash the goods may be redyed in the same jig, preferably with a one or two percent solution of a substantive or direct color of a different shade. After this they may be washed, dried and finished in the usual manner. If it is desired to have the filling threads undyed and left a white in a contrasting color to the dyed warp the last step of dyeing the fabric with a direct color may be dispensed with. If it is desired to dye the filling threads a faster color then they may be dyed with a direct color in a contrasting shade, it is obvious that the filling threads may also prior to weaving be similarly treated with a different type of indigosol such as indigosol helio. The fabric is woven in the usual manner and later on passing the fabric through acid, a blue dyestuff will be developed on the warp and a helio dyestuff will be dyed on the filling, thus as explained eliminating two of the five steps hitherto necessary in dyeing of this description.

It is obvious that by simultaneously treating the warp in the slasher box with a size and with a first step of a two step dyeing process, each of which has no appreciable effect on the functioning of the other, weaving the cloth in the usual manner with the filling and treating the fabric with the second step of a two step dyeing process, which acts on the prepared warp to form the dye thereon, that it reduces the cost of manufacturing an all cellulose textile fabric in contrasting colors by the cost of one entire step in the process, as hitherto explained, namely by the separate step by treating the warp separately with the first step of the two step dyeing process. It is apparent that I have provided a process which may be readily put in the cotton mills without extra equipment and that I have shown for the first time a method of dyeing cellulose fabrics in contrasting colors with colors faster than any hitherto used for this purpose.

As explained, my invention broadly includes the step in the process of manufacturing an all cellulose textile fabric having component sets of warp and filling threads of contrasting colors, which comprises, treating before weaving one of said component sets of threads with a dye ingredient of a two step dyeing process in any stage in the process of manufacture thereof or both sets with a different dye ingredient of a two step dyeing process. Where this is done other than in the size bath however, it is obvious that the cotton mills will have to be provided with additional tanks or other equipment. Where it is desired to thus treat the warp or the filling threads other than in the slashing process they may be treated in exactly the same fashion as hitherto explained with the same

strength solutions omitting the addition of the size to the first step.

It is obvious that in place of treating the entire warp or filling with the first step of a two step dyeing process only parts of them may be so treated and I therefore employ the phrases in the claims "component sets of warp and filling threads" to include the entire warp or filling threads or any desired part thereof.

10 I employ the words "cellulose textile fabric" to include an all cotton fabric, or a fabric made from the type of rayons which contain substantially the same percentage of cellulose as cotton or a greater percentage of cellulose 15 and which have substantially the same affinity for the same types of dyestuffs as cotton namely, viscose rayon, cupra-ammonium rayon and chardonet rayon, etc. entirely or mixed with cotton.

20 I employ the word "weave" in the claims in its broad sense as defined in Webster's Dictionary of 1866 which defines it as follows: 1. "To unite, as threads of any kind, in such a manner as to form a texture; to entwine or 25 interlace into a fabric as to weave wool, silk and the like; hence, to unite by close connection or mixture, to unite intimately . . . 2. To form as cloth, by interlacing threads; to compose, as a texture of any kind, by putting together textile materials; hence, to form 30 into a fabric; to compose."

It is understood that my invention is not limited to the specific processes described and that various deviations may be made therefrom without departing from the spirit and 35 scope of the appended claims.

What I claim as new and desire to secure by Letters Patent is:

1. The herein described improved process 40 of manufacturing an all cellulose textile fabric having component sets of warp and filling threads of contrasting colors, which comprises treating before weaving one of said component sets of threads with the first 45 step of a two step dyeing process, treating before weaving the other component set of threads with a different first step of a similar two step dyeing process, then weaving said prepared component sets to form the fabric, 50 and after-treating the fabric with the second common step of the two step dyeing process which acts upon the one prepared component set to form a dye thereon and which acts upon the other differently prepared component set to form a dye of a different shade and color thereon.

2. The herein described improved process 60 of manufacturing an all cellulose textile fabric in contrasting colors which comprises simultaneously treating the warp in the slashing process with a size and with a preparatory ingredient of a two step dyeing process, each of which has no appreciable effect on the functioning of the other, treating the filling 65 threads with a different preparatory ingredient of a

similar two step dyeing process, weaving the fabric in the usual manner and treating the fabric with the second common step of the two step dyeing process which acts on the prepared warp to impregnate it with a dye and which acts on the prepared filling to impregnate it with a dye of a different color and shade.

3. The herein described improved process 70 of manufacturing an all cellulose textile fabric having component sets of warp and filling threads of contrasting colors, which comprises treating before weaving one of said sets of threads with a mordant, treating before weaving the other component set of threads with a different mordant, then weaving said prepared component sets to form the fabric, and after treating the fabric with the second common step of the two step mordant dyeing process, which acts upon the one prepared component set to form a dye thereon and which acts upon the other differently prepared component set to form a dye of a different shade and color thereon.

4. The herein described improved process 75 of manufacturing an all cellulose textile fabric in contrasting colors which comprises simultaneously treating the warp in the slashing process with a size and with a mordant, each of which has no appreciable effect 80 on the functioning of the other, treating the filling with a different mordant, weaving the cloth in the usual manner and treating the fabric with the second common step of the two step mordant dyeing process, which acts on the prepared warp to impregnate it with a dye and which acts on the prepared filling to impregnate it with a dye of a different shade and color.

5. An all cellulose textile fabric in the gray state made up of interwoven warp and filling threads, the warp threads being impregnated with a size and with the ingredients of the first step of a two step dyeing process and the filling threads being impregnated with the ingredients of the first step of a different two step dyeing process.

6. An all cellulose textile fabric in the gray state made up of interwoven warp and filling threads, the warp threads being impregnated with a size and with a mordant and the filling threads being impregnated with a different mordant.

In testimony whereof I affix my signature.

JOHN C. WATSON.

120

125

130